

## [54] GRAY IRON

[75] Inventors: **Charles Defranco**, Zele; **Jan Van Eeghem**, Deurle, both of Belgium

[73] Assignee: **Centre de Recherches Scientifiques et l'Industrie des Fabrications Metalliques, en abrégé, C.R.I.F.**, Brussels, Belgium

[22] Filed: **Dec. 15, 1971**

[21] Appl. No.: **208,489**

## Related U.S. Application Data

[63] Continuation of Ser. No. 797,622, Feb. 7, 1969, abandoned.

## [30] Foreign Application Priority Data

Feb. 13, 1968 Belgium ..... 710679

[52] U.S. Cl. .... 75/124, 75/130 R, 75/130

[51] Int. Cl. .... C22c 37/00

[58] Field of Search..... 75/123 CB, 124, 130 R

## [56]

## References Cited

## UNITED STATES PATENTS

|           |         |                 |            |
|-----------|---------|-----------------|------------|
| 2,793,114 | 5/1957  | Moore .....     | 75/130     |
| 2,885,284 | 5/1959  | Moore .....     | 75/124     |
| 1,515,244 | 11/1924 | Early.....      | 75/130 R X |
| 2,134,905 | 11/1938 | Bampfylde ..... | 75/130 R X |
| 2,950,187 | 8/1960  | Ototani .....   | 75/124 X   |
| 3,433,685 | 3/1969  | Albertzart..... | 148/35     |

Primary Examiner—L. Dewayne Rutledge

Assistant Examiner—J. M. Davis

Attorney, Agent, or Firm—Hubbell, Cohen & Stiefel; Sheldon Palmer

## [57]

## ABSTRACT

High strength low hardness gray iron consisting essentially of about 1 – 3 percent aluminum, 2 – 4 percent carbon, up to 1% silicon and the balance iron, said gray iron having been inoculated with a minimum of 0.3 percent of an inoculant alloy, the active inoculant of which is selected from the group consisting of calcium, barium and strontium.

12 Claims, 3 Drawing Figures



SHEET 1 OF 2



FIG. 1.



FIG. 2.

INVENTORS

CHARLES DEFARNO  
JAN VAN EEGHEMBy *John DeFranco*

ATTORNEYS



FIG. 3.

INVENTORS

CHARLES DEFRENCO  
JAN VAN EEGHEMBY *James D. Mullings*  
ATTORNEYS

**GRAY IRON**  
**CROSS-REFERENCE TO RELATED APPLICATIONS**

This application is a continuation of application, Ser. No. 797,622, filed Feb. 7, 1969, now abandoned.

The present invention relates to gray iron.

The gray irons actually known as "high strength gray irons with lamellar graphite" have relatively low carbon (2.6 to 3.2 percent) and silicon (1 to 1.5 percent) contents.

The tensile strength of these known irons, measured on a 30mm standard test-bar rarely exceeds 45 kgf/mm<sup>2</sup>, whereas their Brinell hardness may be as high as 320 Brinell.

To attain this high strength, it is generally necessary to add costly alloying elements such as copper, nickel, molybdenum and/or chromium, and to subsequently inoculate the liquid iron.

Furthermore, as a result of their low carbon and silicon contents these known high strength cast irons also present the disadvantage of a rather high tendency to white chilling. The danger of unmachinable white iron formation thus increases with the decreasing wall thickness of the casting.

Furthermore due to their high hardness, the machinability of the known high strength cast irons is rather poor.

The production of cast iron based on iron carbon and aluminum, with little or no silicon was proposed more than 30 years ago.

However, such irons were cast in the non-inoculated state, and their properties were inferior to those of the classical silicon cast irons.

Present knowledge concerning the inoculation mechanism enables one to give a plausible explanation to this phenomenon.

Indeed, due to the high deoxidizing power of aluminum the oxygen content of high aluminum irons, whether it is dissolved as FeO particles or combined with silicon as SiO<sub>2</sub> inclusions, is almost negligible. This means that silicon particles, which act as natural nuclei in normal gray silicon-bearing irons are absent in high aluminum cast irons, and thus, these known but non-inoculated cast irons have a high chilling tendency and tensile properties which are not superior to, and may even be inferior to those of silicon irons.

The present invention is a new and improved alloy, having properties which are not present in irons where aluminum is used with medium or high silicon contents (which are normal in classical silicon irons) nor in irons where high silicon contents are used without aluminum even when inoculated with an alloy containing calcium, barium or strontium. For this purpose, the cast iron according to the invention is characterized by the fact, that on the one hand it contains aluminum as a graphitizing element, and on the other hand it is inoculated.

The tensile strength of the irons according to the invention varies, for irons with lamellar graphite, between 35 and 70 kgf/mm<sup>2</sup>, as a function of wall-thickness and carbon and aluminum contents; their tendency to chilling is almost non-existent.

Belgian patent 563,443 of Dec. 12, 1957 discloses a ferrous alloy which is obtained by simultaneous addition of manganese and aluminum in order to improve the wear and heat-resistance of the iron. The properties of this known iron are considerably different from those of the iron according to the present invention, as

will appear below from a more detailed description of the present iron.

U.S. Pat. No. 2,662,820 of June 30, 1950 suggests the addition of aluminum in the course of elaboration of a gray iron. It must be pointed out however, that this patent concerns the production of a classical gray iron with spheroidal graphite, the purpose of the aluminum being to extend the duration of the effect of the nodulizing agent.

10 According to an advantageous embodiment of the present invention the useful and economical range of the aluminum content lies between 1 and 3 percent.

The silicon content of the cast irons according to the present invention should preferably and advantageously be lower than 1 percent.

In a particular embodiment of the invention, the silicon content is zero. Indeed, as a further advantage of the present invention, the selected from the group consisting of barium and strontium is incorporated in the molten iron by an aluminum containing bearer.

Other details and particularities of the present invention will be apparent from the description given below, by way of non-limitative example, of several embodiments of the invention, with reference to the drawings

25 which show comparative graphs of the physical properties of the cast iron according to this invention, wherein FIG. 1 shows tensile strength plotted against carbon content, FIG. 2 shows tensile strength plotted against silicon content, and FIG. 3 shows tensile strength plotted against Brinell hardness.

The graph of FIG. 1 shows the variation of tensile strength in 30 mm -diameter test bars (ordinate), determined as a function of carbon content (abscissa) on irons containing respectively an average aluminium content of 1.8 percent (curve 1) or 2.5 percent (curve 2) and inoculated by addition of 1% SiCa.

The straight dotted line, 3, in FIG. 1, represents the theoretical tensile strength of classical irons containing 1.5 percent silicon.

40 It is seen therefrom that at the same level of carbon content, the strengths of the aluminum irons inoculated with 1% SiCa, exceed by 10 to 15 kgf/mm<sup>2</sup> the strengths of the classical irons containing 1.5 percent silicon.

45 According to an advantageous embodiment of the present invention, the useful and economical range of the aluminum contents lies between 1 and 3 percent.

FIG. 2 shows the influence of increasing silicon contents (abscissa) on the tensile strength (ordinate) of inoculated aluminum bearing iron cast in test-bars of 3 different diameters.

50 Curve 4 relates to 30 mm -diameter test bars, curve 5 to 20 mm-diameter test bars and curve 6 to 12 mm-diameter test bars.

55 It can be seen that the influence of silicon is slight between 0.4 and 0.8 percent, that the optimum value is about 0.75 percent and that in amounts over 0.9 percent silicon the tensile strength drops very quickly.

The silicon content of the irons according to the present invention should therefore preferably be lower than 1 percent.

According to a particular embodiment of the present invention, the silicon content of the iron as graphitizing element may even be zero, in which case the silicon is replaced totally by aluminum.

60 The influence of increasing manganese, sulfur and phosphorus contents on the properties of a base iron

containing 2.7 percent carbon, 0.45 percent silicon and 1.84 percent aluminum is given below in Table I.

Curve 7 of FIG. 3 shows the relationship between tensile strength (ordinate) and Brinell hardness (ab-

TABLE I

Influence of Mn, S and P on the mechanical properties of aluminum cast iron

| Cast iron | Chill depth in mm | R, kgf/mm <sup>2</sup> |         |         | Impact modulus kgfcm/cm <sup>3</sup> |
|-----------|-------------------|------------------------|---------|---------|--------------------------------------|
|           |                   | ϕ 30 mm                | ϕ 20 mm | ϕ 12 mm | HB ϕ 30 mm                           |
| % Mn      |                   |                        |         |         |                                      |
| A         | .35               | 2                      | 51.3    | 53.6    | 55.2                                 |
|           | .60               | 3                      | 51.9    | 53.8    | 54.6                                 |
|           | .93               | 3                      | 47.5    | 44.2    | —                                    |
|           | 1.10              | 9                      | 47.5    | 46      | 47.1                                 |
| % S       |                   |                        |         |         |                                      |
| B         | .025              | 1                      | 48.6    | 52      | —                                    |
|           | .038              | 2                      | 46.5    | 51.2    | 51.8                                 |
|           | .051              | 4                      | 49.2    | 51.2    | 53.5                                 |
|           | .079              | 5                      | 43.6    | 48      | 50                                   |
| % P       |                   |                        |         |         |                                      |
| C         | .047              | 2                      | 51.7    | 52.6    | 54.1                                 |
|           | .071              | 2                      | 52.1    | 54      | —                                    |
|           | .112              | 2                      | 51      | 49.2    | 52.3                                 |
|           | .182              | 2                      | 49.2    | 50      | 51.5                                 |

These results show that manganese increases the chill depth and decreases both the tensile strength and the impact modulus, particularly when the manganese content exceeds 0.6 percent.

Sulfur increases the chill depth and decreases both the tensile strength and the impact modulus.

Phosphorus has no influence on chill depth but considerably decreases the impact modulus.

It is thus advantageous to limit the manganese, sulfur and phosphorus contents respectively to the following maximum values: 0.7 percent for Mn; 0.05 percent for S and 0.1 percent for P.

Due to the absence of natural nuclei and in spite of the graphitizing effect of the aluminum, the tendency to ledeburitic solidification of the non-inoculated cast irons according to the invention is very important.

The chill depth of the non-inoculated cast irons varies generally between 20 mm and total chill, although it becomes almost non-existent (0-2 mm) after inoculation.

However, to obtain this result, the amount of inoculating alloy added to the cast iron according to the invention must be more greater than that used for the inoculation of conventional silicon cast irons.

Indeed, while the conventional cast irons are generally inoculated with 0.1 to 0.3 percent of an inoculant, for instance SiCa, the cast irons according to the invention must be inoculated with at least 0.3% SiCa.

Although the properties increase with the amount of added inoculant, it is not justified economically to use more than 2% SiCa.

It must be mentioned that it is not indispensable that the inoculant contain silicon as the bearer of the active inoculating element. On the contrary, in order to avoid the introduction of silicon in the iron, and the accumulation of this element by using foundry returns, it is advantageous to inoculate with alloys of the Fe-Al-Ca type, which do not contain silicon, and which have been specially developed for this purpose.

scissa) of aluminum cast iron. The hollow circles are the results obtained with irons containing 1.8 percent aluminum, whereas the crosses represent the results obtained on irons containing 2.5 percent aluminum, all tests having been performed on cast irons inoculated with 1% SiCa and cast in 30 mm-diameter bars.

For comparison purposes with conventional silicon cast irons, the straight dotted line 8 gives the theoretical relation according to the formula

$$HB = 100 + 4.3 R_t, \text{ where}$$

HB is the Brinell Hardness, and  
 $R_t$  is the Tensile Strength.

The black circles represent the scarce quantitative data given in the literature for conventional high strength gray irons.

As seen from FIG. 3, with the same level of tensile strength, the Brinell hardness of the aluminum cast iron is on the average 50 to 60 Brinell units lower than that of the conventional silicon cast irons.

In spite of the high strengths, the hardness of the cast irons according to the invention is relatively low, which results in machinability which is comparable to, or even better than that of the silicon cast irons.

The cast irons according to the present invention also have the advantage of being made from inexpensive raw materials.

The new cast irons are particularly suited to produce high strength castings and thin-walled castings which have to be machined.

The aluminum contained in these cast irons prevents any mold-metal reactions so that sand adherence is almost unexisting.

The skin of the castings of aluminum cast iron is smoother than the skin of the usual castings of silicon cast iron, which allows a considerable reduction of cleaning costs.

A particularly interesting area of application of the new cast irons is in casting in metal molds.

The castings in conventional silicon irons, cast in metal molds must generally be heat-treated to decompose the carbides which are formed during the rapid cooling in the metal mold.

It has been shown experimentally that due to the very low tendency to chilling of the irons according to the present invention, the castings made in metal molds with these irons, do not have to be heat-treated afterwards.

Two non-limitative examples of the composition of cast irons according to the invention, untreated for nodulizing and cast in bars, are given below.

The hardness and strength tables of in Example 1 give the comparative results of tests for an iron according to the invention which has been inoculated, the silicon content being the sum of the silicon content of the base materials and the silicon content added to the iron as a component of the inoculant, and for the noninoculated base iron, the silicon content of the latter being the silicon content of the base materials.

#### EXAMPLE 1

##### Chemical composition:

|                          |          |           |          |
|--------------------------|----------|-----------|----------|
| non-inoculated base iron | 2.90% C; | 0.09% Si; | 1.85% Al |
| inoculated iron          | 2.70% C; | 0.35% Si; | 1.85% Al |
| inoculation with SiCa:   | 1%       |           |          |

##### Tensile strength in kgf/mm<sup>2</sup>

| $\phi$ 30 mm                                                                  |            | $\phi$ 20 mm   |            | $\phi$ 12 mm   |            |
|-------------------------------------------------------------------------------|------------|----------------|------------|----------------|------------|
| non-inoculated                                                                | inoculated | non-inoculated | inoculated | non-inoculated | inoculated |
| 24.7                                                                          | 50.2       | 38.9           | 52.6       | white iron     | 57.9       |
| non-inoculated                                                                |            |                |            |                |            |
| chill depth in mm:<br>impact modulus: kgfcm/cm <sup>3</sup> : ( $\phi$ 30 mm) |            |                |            |                |            |
|                                                                               |            | 40<br>5.6      |            | 2<br>13.5      |            |

##### Brinell Hardness

| $\phi$ 30 mm   |            | $\phi$ 20 mm   |            | $\phi$ 12 mm        |            |
|----------------|------------|----------------|------------|---------------------|------------|
| non-inoculated | inoculated | non-inoculated | inoculated | non-inoculated      | inoculated |
| 246            | 234        | 295            | 256        | white iron<br>(330) | 280        |

#### EXAMPLE 2

In this example an iron inoculated with 1% Fe-Al-Ca has been added for comparison.

Brinell Hardness of the as cast alloy by about 50 Brinell units.

50 2. A high strength low hardness gray iron consisting

|                                                            | %C   | %Si  | Chemical composition | %Mn  | %P    | %S    | %Al  |
|------------------------------------------------------------|------|------|----------------------|------|-------|-------|------|
| non-inoculated                                             | 3.18 | 0.15 |                      | 0.45 | 0.042 | 0.040 | 2.53 |
| inoculated with SiCa                                       | 3.02 | 0.77 |                      | 0.44 | 0.042 | 0.030 | 2.53 |
| inoculated with Fe-Al-Ca<br>(Fe: 40%; Al: 40%;<br>Ca: 20%) | 3.10 | 0.12 |                      | 0.45 | 0.041 | 0.031 | 2.85 |

| Properties                 | $\phi$ 30 mm   |      | $\phi$ 20 mm |                | $\phi$ 12 mm |            |
|----------------------------|----------------|------|--------------|----------------|--------------|------------|
|                            | non-inoculated | SiCa | FeAl<br>Ca   | non-inoculated | SiCa         | FeAl<br>Ca |
| Tensile strength<br>kgf/mm | 40.1           | 47.6 | 49.8         | 42             | 51.8         | 53.5       |
| Brinell Hardness           | 239            | 241  | 245          | 272            | 285          | 278        |
|                            | non-inoculated |      | SiCa         |                | FeAlCa       |            |
| Chill depth in mm:         | 20             |      | 0.5          |                | 0.5          |            |

In order to obtain certain particular properties, such as corrosion or heat-resistance, beside high strength, various quantities of alloying elements may be added separately or simultaneously to the inoculated iron.

5 One may, for instance add:

Copper : 0 - 6%  
Nickel : 0 - 12%  
Chromium : 0 - 5%  
Molybdenum : 0 - 2%  
Zirconium : 0 - 1%

10 It is to be understood that the invention is not limited to the embodiment herein described and that many changes may be made therein without departing from the scope of the present invention.

15 We claim:

1. A high strength low hardness gray iron consisting essentially of about 1 - 3 percent aluminum, 2 - 4 percent carbon, up to 1 percent silicon and the balance iron, said gray iron having been inoculated with 1 to 20 2 percent of an inoculant alloy, the active inoculant of which is selected from the group consisting of calcium, barium and strontium, said active inoculant being present in the alloy in an amount effective to reduce the

essentially of about 1 - 3 percent aluminum, 2 - 4 percent carbon, up to 1 percent silicon, up to 0.7 percent manganese, and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

3. A high strength low hardness gray iron consisting essentially of about 1 - 3 percent aluminum, 2 - 4 percent carbon, up to 1 percent silicon, up to 0.7 percent manganese, up to 0.05 percent sulfur, up to 0.1 percent phosphorus, and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

4. A high strength low hardness gray iron having a flake graphite structure and consisting essentially of about 1 - 3 percent aluminum, 2 - 4 percent carbon, up to 1 percent silicon and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

5. A high strength low hardness gray iron consisting essentially of about 1 - 3 percent aluminum, 2 - 4 percent carbon, up to 1 percent silicon and the balance iron, said gray iron having been inoculated with 1 to 2 percent of an inoculant alloy selected from the group consisting of SiCa consisting essentially of about 33 percent calcium and the balance being silicon and FeAlCa consisting essentially of about 40 percent iron, 40 percent aluminum and 20 percent calcium.

6. A high strength low hardness gray iron consisting essentially of about 1 - 3 percent aluminum, 2 - 4 percent carbon, up to 1 percent silicon, up to 0.7 percent manganese and the balance iron, said gray iron having been inoculated with 1 to 2 percent of an inoculant alloy selected from the group consisting of SiCa consisting essentially of about 33 percent calcium and the balance being silicon and FeAlCa consisting essentially of about 40 percent iron, 40 percent aluminum and 20 percent calcium.

7. A high strength low hardness gray iron consisting essentially of about 1 - 3 percent aluminum, 2 - 4 percent carbon, up to 1 percent silicon, up to 0.7 percent manganese, up to 0.05 percent sulfur, up to 0.1 percent phosphorus and the balance iron, said gray iron having been inoculated with 1 to 2 percent of an inoculant alloy selected from the group consisting of SiCa consisting essentially of about 33 percent calcium and the balance being silicon and FeAlCa consisting essen-

tially of about 40 percent iron, 40 percent aluminum and 20 percent calcium.

8. A high strength low hardness gray iron having a flake graphite structure and consisting essentially of about 1 - 3 percent aluminum, 2 - 4 percent carbon, up to 1 percent silicon and the balance iron, said gray iron having been inoculated with 1 to 2 percent of an inoculant alloy selected from the group consisting of SiCa consisting essentially of about 33 percent calcium and the balance being silicon and FeAlCa consisting essentially of about 40 percent iron, 40 percent aluminum and 20 percent calcium.

9. In a cast gray iron article having a chill depth in mm. of between about 0.5 and 2, said article consisting essentially of about 1 - 3 percent aluminum, 2 - 4 percent carbon, up to 1 percent silicon and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

10. In a cast gray iron article having a chill depth in mm. of between about 0.5 and 2, said article consisting essentially of about 1 - 3 percent aluminum, 2 - 4 percent carbon, up to 1 percent silicon, up to 0.7 percent manganese, and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

11. In a cast gray iron article having a chill depth in mm. of between about 0.5 and 2, said article consisting essentially of about 1 - 3 percent aluminum, 2 - 4 percent carbon, up to 1 percent silicon, up to 0.7 percent manganese, up to 0.05 percent sulfur, up to 0.1 percent phosphorus, and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

12. In a cast gray iron article having a flake graphite structure and a chill depth in mm. of between about 0.5 and 2, said article consisting essentially of about 1 - 3 percent aluminum, 2 - 4 percent carbon, up to 1 percent silicon and the balance iron, said gray iron having been inoculated with 1 to 2 percent of an inoculant alloy, the active inoculant of which is selected from the group consisting of calcium, barium and strontium, said active inoculant being present in the alloy in an amount effective to reduce the Brinell Hardness of the as cast alloy by about 50 Brinell units.

\* \* \* \* \*

UNITED STATES PATENT OFFICE  
CERTIFICATE OF CORRECTION

Patent No. 3,798,027 Dated March 19, 1974  
Inventor(s) Charles Defrancq et al.

It is certified that error appears in the above-identified patent and that said Letters Patent are hereby corrected as shown below:

Title page, left side, alongside the word "inventors:" "Charles Defrancq" should read -- Charles Defrancq --; alongside the word "Assignee"; "Centre de Recherches Scientifiques et l'Industrie des Fabrications Metalliques, en abrege, C.R.I.F.," should read -- Centre de Recherches Scientifiques et Techniques d l'Industrie des Fabrications metalliques, en abrege, C.R.I.F., --. Column 2, line 18, "the selected" should read -- the active inoculating element selected --. Column 2, line 19, "of barium and strontium" should read -- of calcium, barium and strontium --. Column 5, line 13, "tables of in" should read -- tables in --. Column 5, Example 2, "Tensile strength kgf/mm" should read -- Tensile strength  $\text{kgf/mm}^2$  --. Column 6, line 2, "beside" should read -- besides --; Column 6, line 19, claim 1: "innoculated" should read -- inoculated --.

Signed and sealed this 17th day of September 1974.

(SEAL)

Attest:

McCOY M. GIBSON JR.  
Attesting Officer

C. MARSHALL DANN  
Commissioner of Patents